

## UNITED STATES PATENT OFFICE

2,302,352

## REFINING MINERAL OILS

Henry G. Schutze, Baytown, Tex., assignor to  
 Standard Oil Development Company, a corpora-  
 tion of Delaware

No Drawing. Application August 4, 1940,  
 Serial No. 351,437

6 Claims. (Cl. 196—30)

The present invention relates to the refining of mineral oils and is especially concerned with the production of an improved quality oil which has been treated with copper-containing reagents for the removal or conversion of objectionable sulfur compounds therefrom. In accordance with the present process, high quality stable petroleum oil products free of objectionable sulfur compounds are produced by treating a feed oil with a copper-containing reagent and then contacting the treated oil with an organic reagent capable of forming stable complex compounds with the copper atoms, thereby depriving the latter of their ability to catalyze deterioration of the oil while in storage.

It is well known in the art to remove sulfur compounds such as mercaptans from crude petroleum oils such as motor fuels, or to convert them into innocuous compounds by an appropriate chemical treatment, generally known as a sweetening operation. The chemical compound generally employed is a doctor solution which comprises a sodium plumbite solution made from a solution of caustic soda in which a definite amount of lead oxide is dissolved. The feed oil is treated with this solution under conditions to convert the mercaptans to the corresponding disulfides and the lead oxide then precipitated by the addition of free sulfur. An objection to this operation is that it is essential that the correct amount of sulfur be added necessary to completely precipitate the lead oxide. If excess sulfur be added it is dissolved in the gasoline and the treated product thus contains objectionable corrosive sulfur, necessitating rerunning or further treatment of the same. If an insufficient quantity of sulfur be added, the treated product will contain dissolved lead oxide which is also very undesirable. Another objection to the doctor sweetening operation is that when adding the correct amount of sulfur the rate of reaction is relatively slow, particularly at the point of equilibrium.

It has therefore been proposed to substitute other sweetening operations employing copper salts as well as salts of the other heavy metals such as mercury, for the purpose of removing objectionable sulfur compounds and converting them into harmless disulfides. A relatively widely used operation of this character comprises treating oils boiling in the motor fuel, kerosene, and Diesel fuel boiling range, with a reagent containing copper in the presence of a chloride, as for example ammonium chloride. This operation is not entirely satisfactory for the reason that although substantially the entire quantity of the copper salt is removed from the treated oil, the relatively small amount which is difficult to remove apparently catalyzes subsequent deterioration of the treated oil. This is particu-

larly the case when the oil being treated contains various organic acids which react with the copper salts. In order to overcome this disadvantage, it has been proposed to further treat the oil, after removal of the copper solution, with a reagent having the ability to entirely free the oil of objectionable copper compounds. A known operation of this character comprises treating the copper-containing oil with an alkali or alkaline earth metal sulfide or carbonate solution.

I have now discovered a process by which sweetening operations utilizing reagents containing copper may be rendered particularly efficient and economical, which will result in the production of a treated oil having a high stability against subsequent deterioration, and which is free of objectionable sulfur compounds. The process of my invention comprises treating a copper sweetened oil after removal of the copper treating solution with a relatively small quantity of an organic compound having a specific molecular structure. The compounds of my invention will react with the copper compound, which will remove the copper as the catalyzing agent. The compounds which are suitable for securing this result are selected from a wide class of materials which may be represented by the following structural formula:



in which R represents hydrogen or alkyl or aryl radical or may represent carbon or some other element which constitutes a member of a ring structure; in which C represents carbon or may be sulfur, oxygen or nitrogen; in which Y represents a radical containing a hydrogen atom that is replaceable by copper; as for example a phenolic OH radical, a mercaptan SH radical, a carboxyl group, or other acidic group; in which X represents nitrogen, oxygen, or sulfur containing at least one "lone pair" of electrons; and in which N represents a numeral from 0 to 2, inclusive. Compounds of this character are for example, picolinic acid, quinolinic acid, o-aminophenol, m-aminophenol, anthranilic acid, glycine, o-hydroxy-benzoic acid, o-carboxylic thiophenol, oxanilic acid, rubanic acid, and o-amino-benzene sulfonic acid. Especially desirable substances comprise compounds which contain the following linkage:



as for example picolinic acid and quinoline-2-carboxylic acid. An especially desirable substance comprises o-amino-benzoic acid, as well

as o-hydroxy-benzoic acid and o-carboxylic thiophenol. My compounds in general are characterized by the fact that there is a sufficient number of carbon atoms between the X and Y group so that upon reaction with the copper atom either five or six member ring compounds will be formed in the following manner:



In general it is preferred that the organic reagent of the present invention be such that the resulting copper ring compound form be insoluble in the oil, and that the oil be filtered in order to remove these compounds.

The amount of the reagent used per volume of copper sweetened oil will vary considerably depending upon the type of the oil and the character of the copper ion present. If the copper ion is present in the oil in the cuprous state, one mole of organic addition agent per mole of copper is necessary for complete reaction, whereas if the copper is present in the cupric state, two moles of inhibitor per mole of copper are required.

Temperature and pressure conditions may be adjusted in a manner adapted to secure a rapid rate of reaction. In general preferred temperature conditions are in the range from about 60° F. to 100° F. and preferred pressures are substantially atmospheric pressure.

In order to further illustrate the invention the following examples are given which should not be construed as limiting the scope of the invention in any manner whatsoever:

#### EXAMPLE 1

Copper naphthenates were added to a hydrocarbon base oil which comprised an acid treated, redistilled and doctor sweetened cracked naphtha. The copper naphthenates were prepared by reacting naphthenic acids having a molecular weight of about 150 with sodium hydroxide to form sodium naphthenates which were then reacted with copper sulfate to produce the copper naphthenates. Approximately 0.001 gram of copper naphthenates per cubic centimeter of oil were dissolved in the base oil. Varying amounts of this oil solution were then added to larger volumes of an identical base oil in order to prepare the solutions appearing in Table I.

Anthranilic acid was then dissolved in pure benzene and the following operations conducted. Three one-gallon samples of the base oil were prepared for storage tests. The initial test utilized a base naphtha to which had been added 5.3 parts per million of copper in the form of copper naphthenates.

The second test utilized a base naphtha to which had been added 5.3 parts per million of copper and 32.16 parts per million of anthranilic acid. The copper anthranilate complex formed on mixing these constituents was insoluble and settled out while standing in storage. In this operation no attempt was made to remove the

insoluble copper anthranilate. The material was left to settle out and remain in contact with the oil during storage and a portion of the oil was removed from time to time by decantation for inspection and the precipitant was not disturbed.

A third operation was conducted in the same manner identical with that of the second operation except that the insoluble complex copper anthranilate was removed from the oil immediately by percolating the oil through a bed of unburned clay. The inspections on the oil from the respective operations, after various periods of storage, were as follows:

Table I

| Op. I |                                                                                                                        | Storage period                                                       | Saybolt color                          | Break-down time <sup>1</sup>                  |
|-------|------------------------------------------------------------------------------------------------------------------------|----------------------------------------------------------------------|----------------------------------------|-----------------------------------------------|
| 20    | 1 Base naphtha plus 5.3 P. P. M. copper.                                                                               | 3-day<br>2-week<br>4-week<br>8-week<br>12-week<br>16-week<br>20-week | 26<br>22<br>20<br>15<br>16<br>16<br>16 | 405<br>255<br>240<br>200<br>210<br>240<br>260 |
| 25    | 2 Base naphtha plus 5.3 P. P. M. copper plus 32.16 P. P. M. anthranilic acid. Precipitate not removed.                 | 3-day<br>2-week<br>4-week<br>8-week<br>12-week<br>16-week<br>20-week | 30<br>30<br>30<br>27<br>26<br>24<br>21 | 360<br>250<br>360<br>360<br>300<br>270<br>360 |
| 30    | 3 Base naphtha plus 5.3 P. P. M. copper plus 32.16 P. P. M. anthranilic acid. Precipitate removed by clay percolation. | 3-day<br>2-week<br>4-week<br>8-week<br>12-week<br>16-week<br>20-week | 30<br>30<br>30<br>30<br>30<br>30<br>30 | 230<br>225<br>265<br>205<br>225<br>180<br>270 |

<sup>1</sup> Test described in Ind. Eng. Chem., vol. 11, page 511 (1933).

From the above it is apparent that the addition of anthranilic acid to a base oil effects a marked improvement in its color stability and in its resistance to the breakdown oxidation itself. It is also to be noted that the oil percolated through clay for removal of the insoluble copper anthranilate complex had an unusually good color stability but had a poor resistance to the breakdown test. The low breakdown characteristic of the clay percolated oil, as confirmed by the following data on base oils free of added constituents, is believed to be due to some phenomena associated with the clay:

Table II

|    | Sample                                    | Storage period                                                       | Saybolt color                          | Break-down time                               |
|----|-------------------------------------------|----------------------------------------------------------------------|----------------------------------------|-----------------------------------------------|
| 55 | Base naphtha percolated through clay.     | 3-day<br>2-week<br>4-week<br>8-week<br>12-week<br>16-week<br>20-week | 30<br>30<br>30<br>30<br>30<br>30<br>30 | 120<br>180<br>240<br>140<br>180<br>150<br>115 |
| 60 | Base naphtha not percolated through clay. | 3-day<br>2-week<br>4-week<br>8-week<br>12-week<br>16-week<br>20-week | 30<br>30<br>27<br>23<br>29<br>30<br>29 | 400<br>330<br>360<br>395<br>180<br>480<br>360 |

#### EXAMPLE 2

In another series of tests the copper naphthenates employed in Example 1 were utilized. However, the organic addition agent comprised crystalline anthranilic acid in one operation and a solution of anthranilic acid in isopropyl alcohol in other operations. In these operations five one-gallon samples of naphtha were prepared for

storage tests. One sample consisted of base naphtha to which had been added 2.65 P. P. M. of copper in the form of copper naphthenates. A second sample consisted of base naphtha to which had been added 2.65 P. P. M. of copper and 16.08 P. P. M. of crystalline anthranilic acid. After settling for two hours, this sample was filtered through two thicknesses of filter paper to remove the insoluble copper anthranilate complex before placing in storage. A third sample consisted of base naphtha to which had been added 2.65 P. P. M. of copper and 16.08 P. P. M. of anthranilic acid dissolved in isopropyl alcohol (0.7 cc. per gallon of oil sample). This sample was settled for three hours and then filtered through filter paper to remove the insoluble copper anthranilate complex before placing the sample in storage. A fourth sample consisted of base naphtha to which had been added 2.65 P. P. M. of copper as copper naphthenate and 11.45 P. P. M. of anthranilic acid dissolved in isopropyl alcohol, the alcohol used being equivalent to 0.5 cc. per gallon of oil sample. This sample was settled for a period of 3.5 hours before filtering to remove the insoluble copper anthranilate complex. The 11.45 P. P. M. of anthranilic acid is the amount just equivalent to 2.65 P. P. M. of copper as copper naphthenates, whereas 16.08 P. P. M. of the acid amounted to a 40% excess over that equivalent to the copper. A fifth sample, prepared as a control, consisted of base naphtha in which had been dissolved 0.7 cc. of isopropyl alcohol per gallon of sample. The storage data on the respective samples are tabulated below:

Table III

| Sample                                                                                                                               | Storage period | Saybolt color | Break-down time |
|--------------------------------------------------------------------------------------------------------------------------------------|----------------|---------------|-----------------|
| Base naphtha plus 2.65 P. P. M. copper.                                                                                              | 3-day          | 21            | 240             |
|                                                                                                                                      | 2-week         | 20            | 360+            |
|                                                                                                                                      | 4-week         | 16            | 270             |
|                                                                                                                                      | 8-week         | 4             | 325             |
|                                                                                                                                      | 12-week        | 0             | 240             |
|                                                                                                                                      | 16-week        | 3             | 315             |
| Base naphtha plus 0.7 cc. isopropyl alcohol per gallon.                                                                              | 20-week        | 6             | 135             |
|                                                                                                                                      | 3-day          | 26            | 285             |
|                                                                                                                                      | 2-week         | 24            | 360+            |
|                                                                                                                                      | 4-week         | 23            | 360             |
|                                                                                                                                      | 8-week         | 21            | 310             |
|                                                                                                                                      | 12-week        | 21            | 240             |
| Base naphtha plus 2.65 P. P. M. copper plus 16.08 P. P. M. crystalline anthranilic acid. Precipitate removed by filtration.          | 16-week        | 21            | 480             |
|                                                                                                                                      | 20-week        | 20            | 360             |
|                                                                                                                                      | 3-day          | 26            | 465             |
|                                                                                                                                      | 2-week         | 30            | 360+            |
|                                                                                                                                      | 4-week         | 30            | 360+            |
|                                                                                                                                      | 8-week         | 29            | 360+            |
| Base naphtha plus 2.65 P. P. M. copper plus 16.08 P. P. M. anthranilic acid in isopropyl alcohol. Precipitate removed by filtration. | 12-week        | 28            | 490             |
|                                                                                                                                      | 16-week        | 28            | 195             |
|                                                                                                                                      | 20-week        | 26            | 360             |
|                                                                                                                                      | 3-day          | 26            | 315             |
|                                                                                                                                      | 2-week         | 28            | 345             |
|                                                                                                                                      | 4-week         | 29            | 360+            |
| Base naphtha plus 2.65 P. P. M. copper plus 11.45 P. P. M. anthranilic acid in isopropyl alcohol. Precipitate removed by filtration. | 8-week         | 29            | 360             |
|                                                                                                                                      | 12-week        | 30            | 360+            |
|                                                                                                                                      | 16-week        | 30            | 315             |
|                                                                                                                                      | 20-week        | 30            | 330             |
|                                                                                                                                      | 3-day          | 26            | 315             |
|                                                                                                                                      | 2-week         | 26            | 360             |

The above data show that the addition of anthranilic acid to a copper-bearing oil, followed by its filtration through a suitable filter for removal of the resultant insoluble complex copper compound, is an effective method for rendering such oil stable against deterioration while in storage.

While this invention has been described with specific reference to the conversion of copper atoms present in oil to stable complex compounds so as to render them incapable of promoting deterioration of the oil while in storage, the process may also be employed for conversion of the atoms of other metals, such as cobalt, nickel, chromium, zinc, silver and cadmium to stable complex compounds for the same purpose.

10 The process of the present invention is not to be limited by any theory or mode of operation but only by the following claims in which it is desired to claim all novelty insofar as the prior art permits.

I claim:

1. The process of stabilizing petroleum oil which has been sweetened with a copper containing reagent, which comprises treating said oil with anthranilic acid to precipitate an insoluble complex copper-containing compound from retained copper salts reacted with said anthranilic acid, and separating said precipitate from the oil.

2. The process as defined by claim 1 in which said petroleum oil comprises an oil boiling in the motor fuel-boiling range.

3. In the process of sweetening a hydrocarbon oil with a copper reagent, the step of stabilizing the sweetened oil to prevent deterioration thereof caused by copper remaining in the sweetened oil, which comprises reacting with said retained copper in the sweetened oil an organic amino-acid to form a stable complex containing the copper in a 5 to 6 membered ring, said amino-acid being characterized by having the nitrogen atom of an amino group linked to the carbon atom of a carboxyl group thru one to two intervening carbon atoms.

4. In a process of sweetening a petroleum oil with copper reagents, the step of stabilizing the sweetened oil to prevent deterioration due to retained oil-soluble copper salts, which comprises adding to said sweetened oil a small quantity of an aromatic amino carboxylic acid in which a trivalent nitrogen constituent of an amino group is linked by a series of 1 to 2 carbon atoms to the carbon constituent of a carboxyl group so that upon reaction of the aromatic amino carboxylic acid with the copper salt, copper is substituted for a hydrogen atom in the carboxyl group and becomes bonded to the nitrogen in the amino group as a constituent of a 5 to 6 membered ring in combination with said aromatic amino acid.

5. The method of stabilizing a hydrocarbon oil treated with a copper salt reagent to prevent deterioration caused by retained oil-soluble copper salts, which comprises reacting said copper salts with an aromatic amino acid wherein trivalent nitrogen of an amino group is linked to the carbon atom of a carboxylic radical through 1 to 2 carbon atoms.

6. The method of stabilizing a hydrocarbon oil to prevent deterioration normally induced by a copper compound left in the oil in sweetening by a copper reagent, which comprises combining copper from said compound into a complex compound with an aromatic aminoacid wherein nitrogen of an amino group and carbon of a carboxyl radical are located in ortho positions.

HENRY G. SCHUTZ